

# United States Patent [19]

Laemmle et al.

[11] Patent Number: 4,775,418

[45] Date of Patent: \* Oct. 4, 1988

[54] PARTING COMPOSITION COMPRISING GLYCEROL TRIOLEATE AND VEGETABLE OIL

[75] Inventors: Joseph T. Laemmle, Murrysville; John Bohaychick, New Kensington, both of Pa.; Willie Lansdale, Newburgh, Ind.

[73] Assignee: Aluminum Company of America, Pittsburgh, Pa.

[\*] Notice: The portion of the term of this patent subsequent to Jan. 6, 2004 has been disclaimed.

[21] Appl. No.: 893,728

[22] Filed: Aug. 6, 1986

## Related U.S. Application Data

[60] Continuation-in-part of Ser. No. 714,539, Mar. 21, 1985, abandoned, which is a division of Ser. No. 454,268, Dec. 29, 1982, Pat. No. 4,522,250.

[51] Int. Cl.<sup>4</sup> ..... B28B 7/36

[52] U.S. Cl. ..... 106/38.24; 106/250

[58] Field of Search ..... 106/38.24, 250; 424/64

## [56] References Cited

### U.S. PATENT DOCUMENTS

|           |         |                       |           |
|-----------|---------|-----------------------|-----------|
| 3,130,159 | 4/1964  | Stedt .....           | 252/31    |
| 3,495,962 | 2/1970  | Norton et al. .....   | 65/26     |
| 3,592,940 | 7/1971  | Quesada .....         | 99/148    |
| 3,819,523 | 6/1974  | Bove .....            | 252/89    |
| 3,914,131 | 10/1975 | Hutchison .....       | 106/268   |
| 4,246,285 | 1/1981  | Van Duzee .....       | 424/358   |
| 4,410,436 | 10/1983 | Holstedt et al. ..... | 252/46.4  |
| 4,634,469 | 1/1987  | Laemmle et al. .....  | 106/38.24 |

### FOREIGN PATENT DOCUMENTS

611431 12/1960 Canada .

Primary Examiner—Amelia B. Yarbrough  
Attorney, Agent, or Firm—Glenn E. Klepac

## [57] ABSTRACT

A parting composition useful for continuously casting aluminum and aluminum alloys and comprising glycerol trioleate and a vegetable oil. Mixtures of glycerol trioleate with castor oil have superior properties compared with parting compositions previously used for continuous ingot casting.

20 Claims, 1 Drawing Sheet



**PARTING COMPOSITION COMPRISING  
GLYCEROL TRIOLEATE AND VEGETABLE OIL**

**CROSS-REFERENCE TO RELATED  
APPLICATIONS**

This application is a continuation-in-part of U.S. application Ser. No. 714,539 filed Mar. 21, 1985, now abandoned, which is a division of U.S. application Ser. No. 454,268 filed Dec. 29, 1982, now U.S. Pat. No. 4,522,250 issued June 11, 1985.

**BACKGROUND OF THE INVENTION**

The present invention relates to a parting composition comprising a mixture of glycerol trioleate and a vegetable oil. The composition is useful in casting ingots of aluminum and its alloys.

In the casting of aluminum and its alloys, it is customary to employ a mold lubricant and parting agent. Satisfactory ingot surface can be obtained only with a lubricant which has the ability to carry high loads at high temperatures. Until the mid-1950s, lard oil was commonly used as a mold lubricant for aluminum ingot casting. Mold design and lubricant application were not sophisticated and lard oil was often applied to molds by brushing or swabbing prior to casting. The principal disadvantages of lard oil is its tendency to harden to a grease-like consistency at approximately 40° F. This precluded its use in modern continuous casting methods where free flowing lubricant is required for cold weather operations. In addition, ingot cooling water interacts with lard oil to produce a grease-like material which can build up on continuous casting belts, interfere with ingot cooling and cause environmental difficulties. With the advent of advanced casting methods including continuous casting, castor oil has replaced lard oil as the most commonly used mold lubricant. Castor oil does not suffer the above-mentioned disadvantages of lard oil. However, pure castor oil is very viscous and difficult to apply to molds in a uniform fashion, especially in cold weather. In addition, pure castor oil is prone to undergo polymerization under casting conditions and deposit varnish-like films on molds and aluminum ingots leading to unsatisfactory surfaces and tears.

In order to perform satisfactorily on an industrial scale, a mold lubricant must meet several important requirements. Among these requirements are a viscosity at room temperature which allows easy and uniform application and a viscosity at mold-ingot interface temperatures sufficient to maintain a stable lubricant film. The lubricant must also have high resistance to thermal degradation. The lubricant must resist polymerization at high temperatures which lead to varnish-like deposits and unsatisfactory ingot surface. The lubricant must separate from ingot cooling water rapidly to avoid environmental contamination in discharge water and to avoid cooling problems in recirculated water. Aluminum ingot casting mold lubricants have generally not been able to satisfy all the foregoing requirements prior to the present invention.

Pure glycerol trioleate performs very satisfactorily as a continuous casting parting composition for aluminum and its alloys. However, at temperatures up to about 300° C., the viscosity of glycerol trioleate is lower than that of castor oil. The low viscosity of glycerol trioleate

has given rise to concern about possible leakage problems, particularly in warm weather.

Ingot casting lubricants are known in the prior art. Smith et al U.S. Pat. No. 3,524,751 claims an aluminum ingot casting lubricant comprising about 20 to 40% by weight of a lower alkyl ester of an acetylated hydroxy acid having 8 to 20 carbon atoms with about 80 to 60% by weight castor oil. A preferred embodiment involves a mixture of 25% n-butyl acetyl ricinoleate and 75% castor oil. This lubricant is marketed under the trade name Lubricin A-1.

Holshouser U.S. Pat. No. 3,034,186 claims an aluminum ingot casting lubricant which consists of boric acid dispersed in a suitable oily base material. In a preferred embodiment, 2 to 6% by weight of boric acid is mixed with lard oil.

It is a principal object of the present invention to provide a mold lubricant for casting aluminum and its alloys having an ambient temperature viscosity which obviates concern about leakage while permitting uniform application and a mold temperature viscosity sufficient to insure an uninterrupted lubricant film.

Related objects of the invention are to provide a lubricant accomplishing the foregoing objectives while at the same time having high thermal stability, good lubricity, rapid separation from ingot cooling water and avoidance of deposits on ingot and mold surfaces.

A further object of the invention is to provide a parting composition containing effective concentrations of additives such as oxidation inhibitors, biocides, copper corrosion inhibitors and the like, all of which are soluble in the composition itself.

Additional objects and advantages of the present invention will become apparent to persons skilled in the art from the following specification.

**SUMMARY OF THE INVENTION**

In accordance with the present invention, there is provided a lubricant having superior properties as a mold lubricant and parting agent in the continuous casting of aluminum and its alloys.

The parting composition has a pour point below about 2° C. and comprises about 65-95 wt% glycerol trioleate and about 5-35 wt% of a vegetable oil containing predominantly unsaturated fatty acids. The content of saturated fatty acids in the oil should be less than about 5 wt% of total fatty acid content, preferably less than about 10 wt% and more preferably less than about 5 wt%. A particularly preferred vegetable oil, castor oil, has nominal saturated fatty acid content of about 3 wt%.

Animal oils such as lard oil are less satisfactory additives than castor oil because animal oils generally contain significant concentrations of glycerol esters of saturated fatty acids. The saturated acid esters in animal oils generally include esters of myristic acid, palmitic acid, and stearic acid. These esters have high pour points thereby making fats containing them unsuitable for use as continuous casting parting compositions.

Castor oil is the preferred vegetable oil to be mixed with glycerol trioleate in the parting composition of the invention. The following are some other suitable vegetable oils: corn oil, linseed oil, olive oil, peanut oil, rapeseed oil, safflower oil, sesame oil, soybean oil, sunflower oil, and tung oil.

The parting composition of the invention preferably has a pour point below about 0° C. Compositions consisting essentially of about 50-95 wt% glycerol triole-

ate, about 5-50 wt% castor oil, and up to about 2 wt% of a copper corrosion inhibitor, oxidation inhibitor, biocide, or mixtures thereof are quite suitable. As used herein, the term "consisting essentially of" leaves the composition open only for inclusion of other ingredients which do not materially affect the basic and novel characteristics of the composition.

A parting composition consisting essentially of about 65-85 wt% glycerol trioleate and about 15-35 wt% castor oil is preferred. A more preferred composition consists essentially of about 70-80 wt% glycerol trioleate and about 20-30 wt% castor oil.

The parting composition may also have a pour point below about 0° C. and consist of about 25-95 wt% glycerol trioleate, about 5-75 wt% castor oil, and up to about 2 wt% of a copper corrosion inhibitor, oxidation inhibitor, biocide, or mixtures thereof. Compositions consisting of about 50-90 wt% glycerol trioleate and about 10-50 wt% castor oil are preferred, and compositions consisting of about 65-85 wt% glycerol trioleate and about 15-35 wt% castor oil are more preferred. As used herein, the term "consisting of" closes the composition to inclusion of materials other than those recited except for impurities ordinarily associated therewith.

The parting composition may also contain effective concentrations of suitable additives such as oxidation inhibitors, biocides and copper corrosion inhibitors. A suitable oxidation inhibitors is 2,6-di-tert-butyl paracresol at a concentration of about 0.05-1 wt% of the composition. One suitable biocide comprises 4-(2-nitrobutyl)morpholine and 4,4'-(2-ethyl-2-nitrotrimethylene)dimorpholine at a total concentration of about 0.001-0.1 wt% (10-1000 ppm). The composition may also include about 0.01 to 2 wt% of a copper corrosion inhibitor such as 2-mercapto benzothiazole. A preferred concentration of such corrosion inhibitor is about 0.025-0.5 wt%.

#### BRIEF DESCRIPTION OF THE DRAWING

The drawing is a graph, showing extrapolated kinematic viscosity as a function of temperature for selected parting compositions.

#### DESCRIPTION OF THE PREFERRED EMBODIMENT

The preferred parting composition of the invention contains glycerol trioleate and castor oil. Glycerol trioleate is a synthetic material sold under the trade name "EMEREST 2423" by Emery Industries of Cincinnati, Ohio, and "CPH-399-N" by C. P. Hall Company of Chicago, Ill. Particularly preferred embodiments of the invention include mixtures of glycerol trioleate and castor oil as mold lubricants and parting agents for casting ingots of aluminum and its alloys. The unusual and surprising properties of glycerol trioleate which allow its use as a superior mold lubricant will become apparent from the following description.

Mold lubricants for ingot casting must have viscosities at ambient temperature which allow them to be pumped easily and deliver a uniform lubricant film through the tiny passageways provided to allow lubricant to flow to the mold. In addition, such lubricants must have a viscosity at mold-ingot interface temperatures to provide a stable uninterrupted lubricant film. Table I gives the viscosities of the commonly used ingot casting lubricants, castor oil and a mixture comprising 75 wt% castor oil and 25 wt% n-butyl acetyl ricinoleate, along with the viscosities of glycerol trioleate and

glycerol trioleate/castor oil mixtures at the standard temperatures of 40° C. and 100° C.

TABLE I

| Lubricant                                       | Mold Lubricant Viscosities |         |                              |
|-------------------------------------------------|----------------------------|---------|------------------------------|
|                                                 | 40° C.                     | 100° C. | Viscosity Index (ASTM D2270) |
| Castor Oil                                      | 260                        | 19.8    | 97                           |
| 25% n-butyl acetyl ricinoleate + 75% castor oil | 108                        | 12.2    | 120                          |
| Glycerol Trioleate                              | 39.9                       | 8.4     | 203                          |
| 25% Glycerol Trioleate + 75% Castor Oil         | 155                        | 15.5    | 118                          |
| 50% Glycerol Trioleate + 50% Castor Oil         | 93                         | 12.4    | 138                          |
| 65% Glycerol Trioleate + 35% Castor Oil         | 67.9                       | 10.6    | 158                          |
| 75% Glycerol Trioleate + 25% Castor Oil         | 58.7                       | 10.1    | 173                          |

20 The high viscosity of castor oil at 40° C., i.e. 260 cs, renders this material difficult to pump and apply, especially in cold weather. Mixing 75 wt% castor oil with 25 wt% n-butyl acetyl ricinoleate gives a less viscous lubricant but one which has disadvantages in reduced thermal stability and lubricity as will become apparent. Glycerol trioleate has a low 40° C. viscosity, i.e. 39.9 cs. Thus, it can be pumped easily itself or mixed with castor oil to produce a lubricant with enhanced thermal stability and lubricity which has a viscosity tailored for maximum performance in a given delivery system. In addition, glycerol trioleate has a pour point of -8° C. (17° F.) and, therefore, does not produce the problematical grease-like deposits that are associated with lard oil.

25 The viscosity indexes of the above-mentioned lubricants are illustrated in Table I. The viscosity index is related to the change of viscosity with temperature. The higher the viscosity index, the less viscosity is reduced as temperature is increased. The surprising and unexpectedly high viscosity index of 203 for glycerol trioleate indicates that at mold-ingot interface temperatures, glycerol trioleate maintains a viscosity sufficient to provide a stable uninterrupted lubricant film.

30 One of the reasons for superior performance of glycerol trioleate is its favorable ambient temperature viscosity and very high viscosity index. This is further illustrated in a generally accepted extrapolation in FIG. 1 which shows that although glycerol trioleate has viscosity considerably lower than castor oil or a mixture of 75 wt% castor oil and 25 wt% n-butyl acetyl ricinoleate at ambient temperatures, its viscosity and film forming capabilities exceed those of the mixture and approach those of castor oil at mold-ingot interface temperatures.

35 Another property of ingot casting mold lubricants of great importance is thermal stability. This property is a measure of the resistance of the lubricant to vaporization or chemical degradation at high temperatures. Thermal degradation of lubricant to produce vapors in an ingot mold leads to several undesirable consequences. First, lubricants which vaporize more rapidly in the mold require more lubricant to maintain a stable film. This leads to costly higher lubricant usage in addition to greater varnish-like deposits. Second, vapors formed in the mold force separation of the ingot shell from the mold skirt, thereby reducing heat extraction at that point. Thirdly, in casting, where a ceramic header is used, vapors formed in the mold force lubricant into the ceramic header material forcing premature header

deterioration. Lastly, in HDC and FDC casting, vaporization produces erosion of the oil ring and mold skirt leading to cracking of ingot surfaces.

TABLE II

| Lubricant                                                                     | Thermal Stability<br>(As Measured By Thermal Gravimetric Analysis) |         |         | 10      |                                            |
|-------------------------------------------------------------------------------|--------------------------------------------------------------------|---------|---------|---------|--------------------------------------------|
|                                                                               | % Weight Loss Vs.<br>Temperature                                   | 25%     | 50%     | 75%     | Maximum Weight<br>Loss Rate<br>Temperature |
| Glycerol Trioleate                                                            | 752° F.                                                            | 779° F. | 811° F. |         | 802° F.                                    |
| Castor Oil                                                                    | 734° F.                                                            | 768° F. | 801° F. |         | 774° F.                                    |
| Mixture comprising<br>25% n-butyl acetyl<br>ricinoleate and<br>75% castor oil | 635° F.                                                            | 730° F. | 779° F. |         | 766° F.                                    |
| n-butyl acetyl<br>ricinoleate                                                 |                                                                    | 540° F. | 585° F. | 612° F. | 608° F.                                    |

Table II illustrates the thermal stabilities of glycerol trioleate, castor oil, a mixture of 75 wt% castor oil with 25 wt% n-butyl acetyl ricinoleate and n-butyl acetyl ricinoleate as measured by thermal gravimetric analysis. In this generally accepted method of determining thermal stability, a small amount of material is placed on a microbalance in an inert atmosphere, and weight loss with respect to temperature is measured as the temperature is increased at a controlled rate. This method gives the percentage weight loss at a given temperature and the temperature at which the maximum rate of weight loss occurs. Lubricants in which a given percentage weight loss occurs at the higher temperature and in which the maximum rate weight loss occurs at the higher temperature are more thermally stable than lubricants in which these events occur at lower temperatures.

Table II illustrates that glycerol trioleate has the highest thermal stability of the lubricants measured. It should also be noted that n-butyl acetyl ricinoleate has a relatively low thermal stability. Thus, glycerol trioleate can be mixed with castor oil to produce a lubricant with lower ambient viscosity and less tendency to produce varnish while enhancing rather than sacrificing thermal stability, a major improvement over the previously known art. To illustrate the advantages, aluminum alloy 5182 was cast on a commercial size HDC unit (21"×42" ingot) at approximately 4 in/min employing first a mixture comprising 25% n-butyl acetyl ricinoleate and 75% castor oil and then a mixture of 75% glycerol trioleate and 25% castor oil. It required a lubricant flow of about 30 ml/min for the castor oil/n-butyl acetyl ricinoleate mixture to produce a satisfactory ingot, whereas a lubricant flow of about 9 ml/min of the glycerol trioleate/castor oil mixture produced satisfactory ingot.

Still another required property of ingot casting mold lubricants is rapid separation from ingot cooling water. This is required in discharged waste cooling water for environmental reasons. In addition, in systems where cooling water is recirculated, unremoved mold lubricant has a deleterious effect on cooling. Two factors influence the ability of lubricants to separate from water. Firstly, the less dense the lubricant is compared to water, the greater its buoyancy force and the more rapidly separation from water occurs. Secondly, lubricants which have hydroxyl groups capable of hydrogen bonding with water will separate less rapidly. As illustrated in Table III, glycerol trioleate has a lower density than either castor oil or the mixture comprising 25% n-butyl acetyl ricinoleate and 75% castor oil. Glycerol

trioleate contains no hydroxyl groups and, therefore, provides a further advantage over those previously known lubricants.

TABLE III

| Lubricant                                                                     | Oil-Ingot Water Separation |                 |
|-------------------------------------------------------------------------------|----------------------------|-----------------|
|                                                                               | Density (g/ml)             | Hydroxyl Groups |
| Glycerol Trioleate                                                            | 0.908                      | No              |
| Castor Oil                                                                    | 0.961                      | Yes             |
| Mixture comprising<br>25% n-butyl acetyl<br>ricinoleate and<br>75% castor oil | 0.952                      | Yes             |

Other esters of oleic acid, as well as esters of ricinoleic acid and esters of ricinoleic acid in which the 12-hydroxyl group had been acetylated were compared to glycerol trioleate in casting trials. Aluminum 5182 alloy was cast for 4 hours where possible employing each of the test lubricants using an HDC unit casting a 6-inch diameter billet. Lubricant flow was varied from very high to very low rates, and those lubricants in which the flow rate could be varied over the widest interval and still give acceptable ingot were judged to be best. The results, shown in Table IV, illustrate the superior results obtained with glycerol trioleate.

TABLE IV

| Lubricants Listed According to Decreasing Lubricity <sup>(1)</sup> |
|--------------------------------------------------------------------|
| 1. Glycerol Trioleate                                              |
| 2. Castor Oil                                                      |
| 3. Ethyl Oleate                                                    |
| 4. Methyl Oleate                                                   |
| 5. Butyl Ricinoleate                                               |
| 6. Methyl Ricinoleate                                              |
| 7. Methyl Acetyl Ricinoleate                                       |
| 8. Butyl Oleate                                                    |
| 9. Glycerol Triacetyl Ricinoleate                                  |
| 10. Butyl Acetyl Ricinoleate                                       |

<sup>(1)</sup>As determined by HDC Castings of 6-Inch Diameter 5182 Alloy.

Also as illustrated in Table IV, acetylated esters of ricinoleic acid gave extremely poor results. Thus, attempts to lower viscosity and control the varnish deposits attributed to castor oil by adding n-butyl acetyl ricinoleate do so at the expense of thermal stability as illustrated by Table II and at the expense of lubricity as illustrated by Table IV. The lubricant of the present invention enhances both thermal stability and lubricity compared to castor oil.

Preferred compositions of the lubricant include mixtures of glycerol trioleate and castor oil where glycerol trioleate comprises at least 25% of the mixtures. In addition, additives known to persons skilled in the art may be added. Such additives may include biocides, copper corrosion inhibitors and oxidation inhibitors.

A suitable oxidation inhibitor is 2,6-di-tert-butyl paracresol (BHT) at a concentration of about 0.05-1 wt%. A concentration of about 0.5 wt% is particularly preferred. Another suitable oxidation inhibitor comprises about 0.2 wt% propyl gallate, about 0.2 wt% 2,6-di-tert-butyl paracresol and about 0.004 wt% citric acid, based on the weight of parting composition.

When the parting composition is made up in large batches and is likely to be placed into bulk storage for long periods of time before use, it is prudent to add an effective concentration of a biocide. One suitable biocide is sold under the trademark Bioban P1487 by International Minerals & Chemical Corporation. This biocide is effective at concentrations of about 0.001-0.1

wt% (10-1000 ppm). Nominal composition is about 70 wt% 4-(2-nitrobutyl)morpholine, about 20 wt% 4,4'-(2-ethyl-2-nitrotrimethylene)dimorpholine and about 10 wt% inert ingredients.

When the parting composition of the invention is to be used in continuous casting systems having components made of copper that contact the lubricant, it is desirable to add an effective concentration of a copper corrosion inhibitor. For example, small cracks have been found to develop around opening in copper rings where a parting composition lacking such inhibitor is injected. A preferred copper corrosion inhibitor is 2-mercaptop benzothiazole (MBT) in concentrations of about 0.01-2 wt%, preferably about 0.025-0.5 wt%.

A set of laboratory experiments has demonstrated effectiveness of the copper corrosion inhibitor. Results of these experiments are summarized in Tables V and VI.

These tests were performed by sanding copper oil ring material with 150-grit aluminum oxide cloth and cutting the material into small pieces. The pieces were washed with acetone and air dried.

The tests summarized in Table V represent measured weight changes for copper samples after being exposed to 50 milliliter oil samples maintained at elevated temperatures for several hours. The results summarized in Table VI are analyses for copper content of oil samples, both with and without exposure to copper. Content of copper was measured by atomic absorption spectrometry.

TABLE V

Copper Corrosion Tests  
29 Hours At 115° C.

| Oil Sample                                                        | Initial Weight of Copper (gms) | Final Weight of Copper (gms) | Weight Change (gms) | % Weight Change |
|-------------------------------------------------------------------|--------------------------------|------------------------------|---------------------|-----------------|
| 75 wt % glycerol Trioleate + 25 wt % Castor Oil                   | 4.7192                         | 4.7123                       | -0.0069             | 0.15%           |
| Castor Oil                                                        | 4.5163                         | 4.5099                       | -0.0064             | 0.14%           |
| Glycerol Trioleate                                                | 4.6918                         | 4.6885                       | -0.0033             | 0.07%           |
| 75 wt % Glycerol Trioleate + 25 wt % Castor Oil*                  | 4.0141                         | 4.0094                       | -0.0047             | 0.12%           |
| 74.5 wt % Glycerol Trioleate + 25 wt % Castor Oil + 0.5 wt % MBT* | 4.0443                         | 4.0449                       | +0.0006             | 0.01%           |
| Oleic Acid**                                                      | 11.1906                        | 11.1894                      | -0.0012             | 0.01%           |
| Ricinoleic Acid**                                                 | 11.3541                        | 11.3048                      | -0.0493             | 0.43%           |

\*Run 20 hours at 115° C.

\*\*Run 18 hours at 115° C. and approximately twice as much copper.

TABLE VI

Atomic Absorption results

| Oil Sample                                                                  | % Copper |
|-----------------------------------------------------------------------------|----------|
| 1. 75 wt % Glycerol Trioleate + 25 wt % Castor Oil w/Cu                     | 0.009    |
| 2. 75 wt % Glycerol Trioleate + 25 wt % Castor Oil                          | <0.001   |
| 3. Castor Oil w/Cu                                                          | 0.015    |
| 4. Castor Oil                                                               | <0.001   |
| 5. Glycerol Trioleate w/Cu                                                  | 0.005    |
| 6. Glycerol Trioleate                                                       | <0.001   |
| 7. Oleic Acid w/Cu*                                                         | 0.003    |
| 8. Oleic Acid*                                                              | <0.001   |
| 9. Ricinoleic Acid w/Cu*                                                    | 0.24     |
| 10. Ricinoleic Acid*                                                        | <0.001   |
| 11. 75 wt % Glycerol Trioleate + 25 wt % Castor Oil w/Cu**                  | 0.010    |
| 12. 74.5 wt % Glycerol Trioleate + 25 wt % Castor Oil + 0.5 wt % MBT w/Cu** | 0.004    |

\*Run 18 hours at 115° C. and approximately twice as much copper.

\*\*Run 20 hours at 115° C..

The atomic absorption analyses reveal that reactivity with copper is in the following order: Ricinoleic acid-

>Castor Oil>75 wt% Glycerol trioleate+25 wt% Castor Oil>Glycerol Trioleate>Oleic Acid. Ricinoleic acid is a degradation product of castor oil and oleic acid is a degradation product of glycerol trioleate.

5 The above tests also indicate that 2-mercaptop benzothiazole is an effective copper corrosion inhibitor when added to a mixture of glycerol trioleate and castor oil.

## EXAMPLES

10 Some examples of preferred lubricant compositions made in accordance with the invention are as follows:

| Example | Ingredient                       | Content |
|---------|----------------------------------|---------|
| 1       | glycerol Trioleate               | 75.0%   |
|         | Castor Oil                       | 25.0%   |
| 2       | Glycerol Trioleate               | 74.5%   |
|         | Castor Oil                       | 25.0%   |
|         | BHT (oxidation inhibitor)        | 0.5%    |
| 3       | Glycerol Trioleate               | 74.95%  |
|         | Castor Oil                       | 25.00%  |
|         | MBT (copper corrosion inhibitor) | 0.05%   |

The lubricant of Example 1 has been used to successfully cast both DC and HDC ingot. In addition, to the previously mentioned comparison with a castor oil/n-butyl acetyl ricinoleate mixture, the lubricant has been found to cast excellent ingot in a commercial size HDC billet and bar caster which casts 6-inch square ingot, 6-inch diameter ingot and 5-inch by 3-inch rectangular

25

30

ingot. This unit previously employed castor oil and lubricant consumption was reduced 50% by employing the lubricant of Example 1. The lubricant of Example 1 has also been used to cast commercial size ingots of 7050 alloy, 2219 alloy, 6009 alloy and 2024 alloy in a commercial size rectangular DC casting unit. The thick oil coating and buildup on the mold seen with castor oil while operating this unit never occurred when employing the lubricant of Example 1.

The foregoing description of our invention has been made with reference to a few preferred embodiments.

60 Persons skilled in the art will understand that changes and modifications can be made in the invention without departing from the spirit and scope of the following claims.

What is claimed is:

1. A parting composition for the continuous casting of aluminum and its alloys, said parting composition having a pour point below about 2° C. and comprising:

(a) about 65-95 wt% glycerol trioleate, and

65

- (b) about 5-35 wt% vegetable oil wherein the saturated fatty acid content is less than about 15 wt% of total fatty acid content.
2. A parting composition as claimed in claim 1 comprising about 70-80 wt% glycerol trioleate and about 20-30 wt% vegetable oil.
3. A parting composition as claimed in claim 1 comprising about 75 wt% glycerol trioleate and about 25 wt% vegetable oil.
4. A parting composition as claimed in claim 1 wherein said vegetable oil is selected from the group consisting of castor oil, corn oil, linseed oil, olive oil, peanut oil, rapeseed oil, safflower oil, sesame oil, sunflower oil, soybean oil, and tung oil.
5. A parting composition as claimed in claim 1 wherein said vegetable oil is castor oil.
6. A parting composition as claimed in claim 1, further comprising:
- (c) about 0.05-1 wt% of an oxidation inhibitor.
7. A parting composition as claimed in claim 1, further comprising:
- (d) an effective concentration of a biocide.
8. A parting composition as claimed in claim 1, further comprising:
- (e) about 0.01-2 wt% of a copper corrosion inhibitor.
9. A parting composition as claimed in claim 1 wherein the saturated fatty acid content of said vegetable oil is about 10 wt% or less of total fatty acid content.
10. A parting composition as claimed in claim 1 wherein the saturated fatty acid content of said vegetable oil is about 5 wt% or less of total fatty acid content.
11. A parting composition for the continuous casting of aluminum and its alloys, said parting composition having a pour point below about 0° C. and consisting essentially of:
- (a) about 50-95 wt% glycerol trioleate,
  - (b) about 5-50 wt% castor oil, and
  - (c) up to about 2 wt% of a copper corrosion inhibitor, oxidation inhibitor, biocide, or mixtures thereof.

12. A parting composition as claimed in claim 11 consisting essentially of about 65-85 wt% glycerol trioleate and about 15-35 wt% castor oil.
13. A parting composition as claimed in claim 11 consisting essentially of about 70-80 wt% glycerol trioleate and about 20-30 wt% castor oil.
14. A parting composition for the continuous casting of aluminum and its alloys, said parting composition having a pour point below about 0° C. and consisting of:
- 10 (a) about 25-95 wt% glycerol trioleate,
  - (b) about 5-75 wt% castor oil, and
  - (c) up to about 2 wt% of a copper corrosion inhibitor comprising 2-mercaptopbenzothiazole; an oxidation inhibitor selected from the group consisting of 2,6-di-tert-butyl paracresol and a mixture of propyl gallate with 2,6-di-tert-butyl paracresol; a biocide comprising a mixture of 4-(2-nitrobutyl)morpholine and 4,4-(2-ethyl-2-nitromethylene)dimorpholine; or mixtures thereof.
- 20 15. A parting composition as claimed in claim 14 consisting of about 50-90 wt% glycerol trioleate and about 10-50 wt% castor oil.
16. A parting composition as claimed in claim 14 consisting of about 65-85 wt% glycerol trioleate and about 15-35 wt% castor oil.
- 25 17. The parting composition of claim 6 wherein said oxidation inhibitor is selected from the group consisting of 2,6-di-tert-butyl paracresol and a mixture of propyl gallate with 2,6-di-tert-butyl paracresol.
- 30 18. The parting composition of claim 7 wherein said biocide comprises a mixture of 4-(2-nitrobutyl)morpholine and 4,4-(2-ethyl-2-nitrotrimethylene)dimorpholine.
19. The parting composition of claim 8 wherein said copper corrosion inhibitor comprises 2-mercaptopbenzothiazole.
- 35 20. The parting composition of claim 11 wherein said copper corrosion inhibitor comprises 2-mercaptopbenzothiazole; said oxidation inhibitor is selected from the group consisting of 2,6-di-tert-butyl paracresol and a mixture of propyl gallate with 2,6-di-tert-butyl paracresol and said biocide comprises a mixture of 4-(2-nitrobutyl)morpholine and 4,4-(2-ethyl-2-nitrotrimethylene)dimorpholine.

\* \* \* \* \*

UNITED STATES PATENT AND TRADEMARK OFFICE  
CERTIFICATE OF CORRECTION

PATENT NO. : 4,775,418

Page 1 of 2

DATED : October 4, 1988

INVENTOR(S) : Joseph T. Laemmle, John Bohaychick, and  
Willie Lansdale

It is certified that error appears in the above-identified patent and that said Letters Patent is hereby corrected as shown below:

|                               |                                                          |
|-------------------------------|----------------------------------------------------------|
| Col. 1, line 28               | Change "disadvantages" to<br>--disadvantage--.           |
| Col. 2, line 47               | Change "5 wt%" to --15 wt%--.                            |
| Col. 3, line 28               | Change "inhibitors" to --inhibitor--.                    |
| Col. 3, line 65               | Change "Tab1d" to --Table--.                             |
| Table III,<br>Col. 6, line 10 | Change "comprisong" to --comprising--.                   |
| Table IV,<br>Col. 6, line 38  | Change "detrmined" to --determined--.                    |
| Col. 7, line 10               | Change "opening" to --openings--.                        |
| Table V,<br>Col. 7,           | Change "glycerol" (first occurrence)<br>to --Glycerol--. |

UNITED STATES PATENT AND TRADEMARK OFFICE  
CERTIFICATE OF CORRECTION

PATENT NO. : 4,775,418

Page 2 of 2

DATED : October 4, 1988

INVENTOR(S) : Joseph T. Laemmle, John Bohaychick, and  
Willie Lansdale

It is certified that error appears in the above-identified patent and that said Letters Patent is hereby  
corrected as shown below:

Table VI,  
Col. 7, line 49

Change "results" to --Results--.

Col. 8, line 15

Change "glycerol" to --Glycerol--.

Signed and Sealed this

Twenty-first Day of February, 1989

Attest:

DONALD J. QUIGG

Attesting Officer

Commissioner of Patents and Trademarks